

Sept. 29, 1936.

J. B. REBER

2,055,750

WIRE ROPE CENTER

Filed Feb. 18, 1935



Inventor

J. B. Reber

By *Chuck O'hurch*  
His Attorneys

## UNITED STATES PATENT OFFICE

2,055,750

## WIRE ROPE CENTER

James B. Reber, Auburn, N. Y., assignor to Columbian Rope Company, Auburn, N. Y., a corporation of New York

Application February 18, 1935, Serial No. 7,084

4 Claims. (Cl. 117—59)

This invention relates to improvements in centers for wire ropes and particularly to the core around or upon which the several strain carrying wire strands of such a rope are laid.

5 Numerous efforts have heretofore been made to produce a center of this type, which will possess all the desired characteristics, i. e., a center having strength, flexibility, durability, water 10 resistant properties, and the capability of properly conforming to the cross-sectional contour of the space occupied by it within a rope when initially incorporated therein under pressure, while subsequently retaining the cross-sectional shape thus imparted thereto, so as to afford a 15 proper seat for the rope strands without being further compressed. Such prior efforts have resulted in the use of various long vegetable fibers and paper. In the present instance, the long vegetable fibers are used in combination 20 with an adhesive, preferably possessing lubricating properties, but instead of placing a high degree of twist in the fibers such as is necessary to render the center stable, a lesser degree of twist is used and this, in conjunction with the binder, 25 renders the center stable. All binders have a tendency to reduce the softness and flexibility of a mass of vegetable fibers and, if twist alone is relied upon for retaining the shape of the original center, the degree of twist required will result in 30 a compact body of fibers that will not properly lend itself to conforming to the space in which it is confined in the rope. Hence, by relying partially on the twist of the fibers and partially on the binder, a lower degree of twist may be 35 used whereby softness and flexibility is imparted to the center and, by the same token, a less quantity of binder is used, whereby that softness and flexibility is not detrimentally affected.

With these and other objects in view, the invention consists in certain details of construction and combinations and arrangements of parts, all as will hereinafter be more fully described, and the novel features thereof particularly pointed out in the appended claims.

45 In the accompanying drawing—

Figure 1 is a perspective view of a length of wire rope made up with the present center;

Fig. 2 is a perspective view of a length of the center with one end portion laid open to more 50 fully illustrate the preferred construction of center;

Fig. 3 is a perspective view of a length of wire rope with portions of the wire strands removed to illustrate the effect of compressing the center 55 within the rope; and

Fig. 4 is a perspective view illustrating a modified form of center.

In the production of the present center, it is desired that the fibers be brought into association with each other so as to impart a certain 5 softness and flexibility to the mass or body constituting the center. For this reason, they are given only a slight twist, as compared to the degree of twist which would be required to hold the center in shape. As illustrated in the drawing, the fibers, in the form of one or more slivers, are twisted together. Where a plurality of slivers are used, one sliver indicated at 10 may be located centrally of the remaining or outer slivers 11. Preferably, the slivers are twisted together in the condition in which they emerge from the preparation room of the ordinary rope factory, i. e., they are not spun and have practically no twist. The several slivers are brought together by running them into the usual former machine, this operation usually imparting the desired twist to them.

As before mentioned, the twist given the sliver or slivers is not sufficient to hold the center intact. For this reason, the fibers or slivers have 25 incorporated therein an adhesive or binder, preferably of a type possessing lubricating properties. Latex compounds are one example and probably preferred, although other colloid rubber compounds or synthetic resins can be used with good 30 results. One precaution to be taken is not to use such a quantity of binder as will seriously detract from the softness and flexibility of the completed center. This is readily prevented in the present invention, because the twist given the 35 fibers in the former aid to a certain extent in retaining the center intact, so that a reduced quantity of binder will suffice, as compared to the quantity that would be required if no twist is given the fibers. In other words, the combined 40 action of the twist and binder hold the center intact and by using a low degree of twist and a reduced quantity of binder, maximum stability is obtained without detracting from the softness, pliability and flexibility of the finished center. 45

The binder can be incorporated in one or more of the slivers by running them through a bath preliminary to passing them through the binder. Satisfactory results have been obtained by running the inner sliver through such bath, the 50 binder being forced into the surrounding fibers or slivers by compression of center. Another arrangement is illustrated in Fig. 4, wherein elongated fibrous elements, such as yarns 12, impregnated with a suitable binder are run into the 55

several slivers, the binder permeating the fibers surrounding such yarns.

It will be appreciated that the disposition of the slivers in a center is not limited to the particular arrangement shown. As stated, one or more slivers can be brought together into a unit such as shown and if a still larger center is desired, a plurality of such units may be formed up into a center. It will also be appreciated that the degree of twist given the fibers and the quantities of binders used will vary somewhat, dependent on the type of fiber, some fibers being softer than others. In each instance, the amount of twist and the quantity of binder is regulated to produce a center of sufficient softness to permit the wire strands 13 of the rope to seat themselves around the same, deforming the center by producing spirally extending depressions 14 therein by reason of the compressive strains imposed upon the center in the laying on of the strands. This original compression of the center reduces the latter to a substantially incompressible mass, the cross sectional dimension of the center at that time being such as to prevent the strands inflicting injury upon one another by undue contact with each other. At the same time, the increased flexibility of a center of the present construction and the lubricating value of the binder insures lengthy service of the center and, consequently, of the rope. Where a latex compound is used, the fibers of the center are thoroughly water-proofed, thus further assuring prolonged life for the center.

What I claim is:

- 35 1. In a wire rope comprising a plurality of twisted strands, a center member composed of a multiplicity of elongated unspun fibers extending longitudinally of the center with a low degree of twist whereby softness and flexibility is imparted to said center and a stabilizing agent incorporated in said center, the volume of stabilizing agent present being such that the softness and flexibility of the finished center will permit the mass of fibers constituting the center to properly adapt 45 itself to the cross sectional contour of the space enclosed by the wire strands of a rope and to the flexing of said rope, said center being reduced to a substantially incompressible mass within said rope.
- 50 2. In a wire rope comprising a plurality of twisted strands, a center member composed of a mass of elongated unspun vegetable fibers arranged longitudinally of the center with a low

degree of twist whereby softness and flexibility are imparted to said center, and a lubricating agent incorporated with said fibers and possessing adhesive properties capable of retaining the unspun fibers in a substantially cylindrical body 5 prior to incorporation of the center in a wire rope, the quantity of said agent present in the center being sufficient to retain in said center a degree of softness and flexibility that will facilitate said center flexing with a wire rope in which 10 it is incorporated and will permit said center to readily conform to the cross sectional contour of the space defined by the strands of a wire rope, said center being reduced to a substantially incompressible mass within said rope and said lubricant having ready access to said strands. 15

3. In a wire rope composed of a plurality of twisted strands, a center member formed of a plurality of slivers of vegetable fibers extending spirally and longitudinally of the center, said fibers of themselves constituting an unstable mass due to lack of twist, and an adhesive incorporated in said center, said adhesive and the spiral disposition of the slivers conjointly rendering said center stable whereby the softness and flexibility imparted to the center by the low degree of twist is not materially reduced by the quantity of adhesive required to stabilize the center and whereby said center will readily conform to the cross sectional contour of the space defined by the strands of a wire rope, said center being reduced to a substantially incompressible mass within said rope but capable of flexing with the strands of the rope. 20 25 30

4. In a wire rope composed of a plurality of twisted strands, a center member formed of a plurality of groups of elongated, unspun vegetable fibers twisted together to form a substantially cylindrical mass, the degree of twist alone being insufficient to render said mass stable, and a water-resistant binder incorporated in said mass, said binder in conjunction with the twist of the fibers rendering said mass stable, whereby a minimum quantity of binder is required, the softness and flexibility of the mass due to the lack of twist 40 therein being retained to facilitate the cylindrical mass conforming to the space defined by the strands of a wire rope in which said center is incorporated and to facilitate said center flexing 45 with the strands of said rope, said center being reduced to a substantially incompressible mass within said rope. 50

JAMES B. REBER.